

# United States Patent [19]

Habermann et al.

[11] Patent Number: 4,668,347

[45] Date of Patent: May 26, 1987

[54] ANTICORROSION COATED RECTIFIER  
METALS AND THEIR ALLOYS

[75] Inventors: Clarence E. Habermann; David S.  
Garrett, both of Midland, Mich.

[73] Assignee: The Dow Chemical Company,  
Midland, Mich.

[21] Appl. No.: 804,721

[22] Filed: Dec. 5, 1985

[51] Int. Cl.<sup>4</sup> ..... C25D 5/44

[52] U.S. Cl. ..... 204/33; 204/32.1;  
204/56.1; 204/58; 204/58.4

[58] Field of Search ..... 204/58, 58.4, 56.1,  
204/32.1, 33, 56 M

## [56] References Cited

### U.S. PATENT DOCUMENTS

|           |        |                   |          |
|-----------|--------|-------------------|----------|
| 2,880,148 | 3/1959 | Evangelides       | 204/35   |
| 3,834,999 | 9/1974 | Hradcovsky et al. | 204/58.4 |
| 3,956,080 | 5/1976 | Hradcovsky et al. | 204/58.4 |
| 4,184,926 | 1/1980 | Kozak             | 204/58.4 |

### FOREIGN PATENT DOCUMENTS

543726 3/1942 United Kingdom ..... 204/56 M

### OTHER PUBLICATIONS

Chemical Abstracts, vol. 75, 1971 p. 422 104365n Anodizing in Fluoroboric Acid solutions.

Primary Examiner—R. L. Andrews

[57]

### ABSTRACT

Metals and alloys of metals which have the property of electrolytic rectification can be coated with an anticorrosive coating by immersion in a strongly alkaline aqueous bath comprising a water soluble fluoride, a water soluble iron salt, and mixtures thereof by the application of a sufficiently high voltage to obtain spark discharge at the surface to be coated, said potential being applied between the metal or alloy to be coated utilized as an anode and a cathode immersed in the aqueous bath. A durable coating is thereby applied to the surface of said metals or alloys thereof which is resistant to a corrosive salt spray environment.

15 Claims, No Drawings

ANTICORROSION COATED RECTIFIER METALS  
AND THEIR ALLOYS

BACKGROUND OF THE INVENTION

1. Field of the Invention

This invention relates to an electrolytic process for the formation of a hard, protective film on the surface of a rectifier metal or alloy thereof.

2. Description of the Prior Art

One of the primary problems associated with the extensive use of magnesium and aluminum is the tendency of these metals to corrode especially when exposed to an environment where an alkali metal halide such as sodium chloride is present alone or in combination with water. A well known process for providing a protective coating for aluminum is the process of anodization. This process has been used to a limited extent with magnesium but the coatings obtained are not 20 highly resistant to attack by corrosive agents such as acids or alkalis, particularly aqueous sodium chloride.

A process is disclosed for anodizing, in fluoroboric acid solutions, aluminum and alloys of aluminum, as described in Chemical Abstracts 75:104365n. A solution containing 0.1 to 2.5% fluoroboric acid was utilized to anodize aluminum and aluminum alloys at a temperature of 0° to 30° Centigrade. A film of high breakdown voltage/thickness ratio was obtained on aluminum indicating a film of compact structure similar in nature to a barrier film. Increased anodizing temperature had an effect similar to higher concentration and increased the deposition of the oxide film. The behavior of the coated aluminum alloys was less satisfactory than the pure metal in resisting corrosion under salt fog conditions.

In U.S. Pat. No. 3,834,999 there is disclosed the electrolytic production of glassy layers on metals and alloys in order to improve corrosion resistance of said metals and alloys wherein the layers are applied by the anodization of the metals and their alloys in anodization baths containing anions such as tungstate, phosphate, arsenate, stannate, molybdate, borate, chromate, and dichromate. The minimum voltage disclosed as useful in the electrolytic anodization of metals or their alloys is about 600 volts.

In U.S. Pat. No. 4,184,926, there is disclosed an anti-corrosive coating for magnesium and its alloys which is capable of withstanding the action of strong acids and alkalis prepared by first treating the metal or the alloy thereof with an aqueous solution of hydrofluoric acid to form a fluoromagnesium first layer on the metal surface. After rinsing off the hydrofluoric acid, the metal or alloy is immersed in an electrolytic bath containing an aqueous solution of an alkali metal silicate and an electrical potential is applied between the metal as an anode and a cathode, also immersed in the bath, in order to apply a uniform silicate layer over the first layer on the metal.

In U.S. Pat. No. 3,956,080, there is disclosed a process for coating a rectifier metal such as aluminum or magnesium, said coating being resistant to attack by chemical agents. The protective coating is applied by immersing the metal in a bath containing an alkali metal silicate and applying an electrical potential between the metal, utilized as an anode, and a cathode also immersed in the bath. This reference teaches away from the use of such undesirable ions as bromide, fluoride, iodide, chloride,

sulphate, nitrate, and cyanide to form the protective coating.

SUMMARY OF THE INVENTION

5 A rectifier metal article or alloy thereof can be coated with a corrosion resistant fluoride or iron containing coating by an electrolytic process utilizing a strongly alkaline aqueous bath comprising at least one water soluble fluoride or iron salt or mixture thereof. The 10 coating is applied by establishing a potential difference of at least about 50 volts between said rectifier metal or alloy thereof as an anode immersed in said bath and a cathode also immersed in said bath. The coatings are 15 resistant to the corrosive effects of acids and alkalis, particularly the corrosive effects of aqueous sodium chloride. Improved anticorrosive coatings are obtained when an aqueous hydrofluoric acid pretreatment is utilized prior to coating the rectifier metal or alloy thereof with the water soluble fluoride or iron salt.

DETAILED DESCRIPTION OF THE INVENTION

A corrosion resistant, hard, uniform adherent coating can be applied to a rectifier metal or alloy thereof by immersing the metal in an electrolytic cell bath containing a water soluble fluoride or iron salt or mixture thereof and establishing a potential difference of at least about 50 volts between said rectifier metal or alloy thereof as an anode and a cathode immersed in said bath. The bath is made strongly alkaline by incorporating 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 10000 10005 10010 10015 1

In order to form the coating on the rectifier metal, this metal is made the anode in an electrolytic cell so that the metal itself is at a positive potential. Improved anticorrosive coatings are obtained when an aqueous hydrofluoric acid pretreatment is utilized prior to coating the rectifier metal or alloy thereof with the water soluble fluoride or iron salt. The cathode of the electrolytic cell can be any suitable material which will not substantially dissolve in, react with or otherwise interfere with the deposition of the surface coating on the rectifier metal anode. Such cathode materials include iron, stainless steel, nickel, graphite, or other conducting forms of carbon and mixtures containing conductive carbon, magnesium, chromium, silicon, mercury, sodium-mercury amalgam, platinum, gold, rhodium, silver, palladium, iridium, osmium, cobalt, and the like. Certain types of cathodes can also be enclosed in permeable glass or other poorly conductive material. Preferred cathode materials for use herein are iron and stainless steel. One skilled in the art will appreciate that the cathode of the electrolytic cell need not be in the form of an electrode element immersed in the electrolyte bath but can in fact comprise the container for the electrolyte bath. Similarly the rectifier metal can be utilized as the container for the electrolyte and a cathode in the form of a rod, bar, sheet, grid, or other suitable form of metal can be dipped into the electrolyte bath.

It should be noted that a high voltage difference is utilized in the electrolytic cell in the process of coating a rectifier metal, the cathode being made of a different metal from that of the metal to be coated. The electrical potential difference in current density applied to cause deposition of a protective coating in accordance with the invention can vary according to factors such as composition of the electrolyte bath, the rectifier metal, the type of coating desired, and the like. Generally, the anode and cathode are connected to an electrical power source and the voltage across the bath is gradually increased until a spark discharge occurs at the anode surface. The voltage is further increased until a coating of the desired thickness has formed. Alternating current can be used because of the rectification effect of the rectifier metal anode. Use of direct current is preferred. When the potential difference reaches or exceeds about 50 volts, a spark discharge occurs.

To form the corrosion resistant layer on a rectifier metal substrate of the invention, the voltage is applied starting at a low value and gradually increased. Initially, the rectifier metal is oxidized but when the voltage reaches about 50 volts deposition of the coating starts. As the voltage is increased, further spark discharges appear on the surface of the rectifier metal anode. The temperature of the spark discharges may be as high as 1,500° centigrade. It is believed that the high temperature resulting from the discharge melts the coating being applied to the rectifier metal surface and insures that a homogeneous, pore free coating on the surface of the metal is formed. The thickness of the coated layer depends upon the current density, the duration of the coating process and the concentration of the electrolyte bath.

The oxidation of the surface of the rectifier metal reaches a maximum generally within a few seconds from the initial immersion of the rectifier metal in the bath and the establishment of the potential difference of at least 50 volts between said rectifier metal and the cathode in the electrolyte bath. The voltage must then be increased in order to maintain a flow of current and

efficient deposition of the anticorrosive coating of the invention. Depending upon the length of time utilized to deposit the coating on the rectifier metal and upon the voltage used for the deposition, anticorrosive layers up to about 2 millimeters in thickness can be readily achieved. A coating thickness of about 0.001 millimeter to about 2 millimeters provides suitable anticorrosion properties when the coated rectifier metal is exposed to a salt spray environment.

In applying a coating to a rectifier metal in accordance with the process of the invention, the current density is generally held in a range of about 250 to about 500 millamps per square centimeter by adjustment of the voltage. To prepare a satisfactory coating the voltage may need to be raised to at least about 500 volts and may go as high as about 1,000 volts. At the higher end of the voltage range, the surface of the coating can become rough. In any case the coating does not become porous.

The optimum electrolytic cell bath temperature for coating a rectifier metal in accordance with the process of the invention is about 30° to about 90° centigrade, preferably about 50° to about 60° degrees centigrade. Since substantial amounts of heat can be generated by the process it may be necessary, if the anode is large in size, to use auxiliary means of cooling the bath.

After the voltage is applied during the coating process of the invention so as to obtain spark discharge and the coating has been formed on the rectifier metal, the power is maintained until the desired coating thickness is formed. Then the power is removed from the anode and the cathode and the coated rectifier metal anode is removed from the bath. Generally the coated rectifier metal is rinsed to remove the highly alkaline electrolytic bath liquid from the surface of the coated metal. The rinsing can take place utilizing plain water. The components of the electrolytic bath include an alkali metal hydroxide generally in the amount of at least about 5 grams per liter but amounts of alkali metal hydroxide up to the saturation level can be used such as up to about 100 grams per liter of alkali metal hydroxide. The preferred alkali metal hydroxide is sodium or potassium hydroxide. Preferred alkali metal hydroxide concentrations for use in the process of the invention are from about 5 grams per liter to about 50 grams per liter.

The strongly alkaline electrolytic cell bath utilized in the coating process of the invention also contains a water soluble fluoride or a water soluble iron salt. The alkali metal hydroxide besides providing an electrolyte functions to provide increased hardness in the coating applied to the rectifier metal. Thus, the use of an increased amount of alkali metal hydroxide in the bath is generally believed to result in an increase of the hardness of the coating applied to the rectifier metal.

The concentration of the water soluble fluoride or water soluble iron salts in said electrolytic cell generally can be about 5 to about 150 grams per liter. Preferably about 10 to about 100 grams per liter is used providing the water soluble salts have solubilities at the higher portions of these ranges. Examples of useful water soluble fluoride salts are the ammonium and the alkali metal fluoroborates, the ammonium and the alkali metal fluoroaluminates, the ammonium and the alkali metal fluosilicates, and mixtures thereof. Examples of useful iron salts are the ammonium or the alkali metal iron cyanides and the ammonium or the alkali metal iron oxalates, and mixtures thereof.

Variations in color as well as other properties of the coating can be provided by the addition of small quantities of other compounds to the electrolytic bath. Compounds which provide anions capable of changing the color of the coating are those compounds of vanadium, arsenic, boron, chromium, titanium, tin, antimony, tungsten, molybdenum or combinations thereof preferably in the form of the alkali metal salts. These compounds are useful in amounts of up to about 50 grams per liter.

Alternatively, said rectifier metal or alloy thereof can be pretreated prior to coating by electrochemical means with an aqueous solution of hydrofluoric acid or an aqueous solution of a fluoride salt. Ammonium fluoride, ammonium bifluoride and the alkali metal fluoride and bifluoride salts are useful.

In order to evaluate the anticorrosive protective action of the coated rectifier metal prepared in accordance with the process of the invention, panels of a magnesium alloy having the composition magnesium 90, aluminum 9, and zinc 1 were coated with various fluoride containing or iron containing coatings. Generally a coating layer of about 0.001 millimeter to about 2 millimeters was utilized. The panels were tested by exposure to an aqueous solution of sodium chloride having a concentration of 5% by weight sodium chloride in accordance with standard test procedure ASTM B-117-73 in which a spray of said sodium chloride aqueous solution is applied at 95° F. to the panel and the sample is evaluated for the percent corrosion at regular intervals.

The following examples illustrate the various aspects of the invention but are not intended to limit its scope. Where not otherwise specified throughout this specification and claims, temperatures are given in degrees centigrade, and parts, percentages, and proportions are by weight.

#### EXAMPLE 1 (CONTROL, FORMING NO PART OF THIS INVENTION)

As a basis for comparison of the coatings applied in accordance with the process of the invention, a panel of magnesium alloy (magnesium 90, aluminum 9, zinc 1) coated with a commercial chromate type corrosion resistance coating was tested in a salt spray environment over a period of seven days (168 hours) and was found to show 5 to 10% corrosion evenly distributed over the surface of the sample.

#### EXAMPLE 2 (CONTROL, FORMING NO PART OF THIS INVENTION)

In order to illustrate the type of coating obtained when anodizing a magnesium alloy in the presence of an aluminate ion a 1.5 inch by 4 inch panel of a magnesium alloy having the composition magnesium 90, aluminum 9, and zinc 1 was polished with No. 1 grit sandpaper and rinsed with acetone thereafter. This panel was spark anodized in an electrolytic bath, the magnesium alloy panel formed the anode in the electrolytic cell and an iron cathode was used as the cathode of the cell. The electrolytic bath contained a solution of sodium hydroxide at a concentration of 40 grams per liter and a solution of sodium aluminate,  $Na_2Al_2O_4 \cdot 3H_2O$ . The potential applied across the cell varied from 70 to 100 volts and 0 to 15 amperes for a period of 10 minutes during which time the coating was applied. A gray, partially crystalline coating was formed on the magnesium alloy. After one week of exposure to aqueous salt spray testing

the coated magnesium panel was corroded to the extent of about 20% upon exposure at 5% by weight sodium chloride and 95° F.

#### EXAMPLE 3

A 1.5 inch by 4 inch panel of magnesium alloy having the composition magnesium 90, aluminum 9, and zinc 1 was sanded utilizing No. 1 grit sandpaper and thereafter rinsed with acetone. The panel was made an anode in an electrolytic cell having an iron cathode and an electrolytic solution containing 40 grams per liter of sodium hydroxide, 20 grams per liter of sodium fluosilicate and 20 grams per liter of sodium silicate ( $Na_2SiO_3 \cdot 9H_2O$ ). The applied potential was 70 volts at 15 amperes over a period of 12 minutes during which time the coating was applied by spark anodization to the magnesium alloy panel. A uniform gray coating was obtained which after rinsing in plain water was tested for corrosion tendency in a salt spray chamber containing a 5% by weight aqueous solution of sodium chloride at a temperature of 95° Fahrenheit. Exposure in the salt spray chamber for a period of 1,484 hours resulted in 2% corrosion of the sample. After a total of 3,500 hours the sample showed 10% pitting corrosion.

#### EXAMPLE 4

Utilizing a similarly treated panel of the same magnesium alloy as used in Example 3, the panel before spark anodizing was pretreated by dipping into 10% aqueous solution of hydrofluoric acid for a period of 2 minutes. Thereafter spark anodization of the panel was carried out utilizing an electrolytic bath solution containing 80 grams per liter of sodium hydroxide and 30 grams per liter of sodium fluosilicate. The coating was applied utilizing a potential of 65 volts and 15 amperes for a period of 14 minutes. It is noted that the amperes decreased to zero over this period. A hard white somewhat uneven coating was obtained which after rinsing was exposed in a salt spray chamber, as described above, for a period of 989 hours. The sample after this time exhibited only 0.5% corrosion. After a total of 2,455 hours the sample showed about 35% corrosion.

#### EXAMPLE 5

Utilizing the same pretreatment in hydrofluoric acid as described in Example 4 and the same magnesium alloy, spark anodization was carried out to apply a coating to the magnesium alloy panel utilizing an electrolytic bath containing 30 grams per liter of sodium fluosilicate, 40 grams per liter of diethylene glycol, and 40 grams per liter of sodium hydroxide. The cathode utilized was of iron. The potential applied was 240 volts at 4 to 6 amperes. This potential did not produce visible sparking but a smooth, white, tough and dense coating was obtained which after rinsing in plain water was exposed to a salt spray chamber, as described above, and found to show less than 0.5% corrosion after a period of 499 hours and after a period of 2,510 hours, less than 10% corrosion was exhibited.

#### EXAMPLE 6

Utilizing the same magnesium alloy, the same pretreatment in hydrofluoric acid, as shown in Example 4, and the same composition of electrolyte bath, the magnesium panel was coated at a potential of 280 volts and 4 to 6 amperes. After rinsing in plain water the coated magnesium alloy was pressed in a hydraulic press at a pressure of  $10^5$  pounds per square inch in order to com-

press and smooth the coating surface. Upon exposure to the salt spray chamber containing 5% sodium chloride at a temperature of 95° Fahrenheit, it was noted that after a period of 499 hours, the sample showed less than 0.5 percent corrosion and after 2,510 hours in the salt spray chamber the sample showed less than 10% corrosion.

#### EXAMPLE 7

Utilizing the same magnesium alloy and the same pretreatment in hydrofluoric acid, as shown in Example 4, a magnesium alloy panel was spark anodized in an electrolyte solution containing 25 grams per liter of sodium aluminate, 25 grams per liter of sodium fluoroaluminate, 16.1 grams per liter of potassium hydroxide, and 62.5 milliliters per liter of diethylene glycol. The spark anodization was carried out utilizing a potential of 320 volts at 4 to 5 amperes over a period of 1 to 2 minutes. After rinsing in plain water the coated sample was subjected to the salt spray chamber, as described above, and found to show 2 to 3% corrosion after a period of 1,816 hours. After a total of 3,864 hours, the coated surface was less than 10% pitted.

#### EXAMPLE 8

Utilizing the same magnesium alloy and the same pretreatment in an aqueous hydrofluoric acid solution, as disclosed in Example 4, a magnesium alloy panel was spark anodized in an electrolyte containing 27.5 grams per liter of sodium fluoroborate, 80 grams per liter of sodium hydroxide, and 6 grams per liter of potassium ferricyanide  $K_4Fe(CN)_6$ . The coating process was carried out utilizing a potential of 5 to 65 volts and 15 amperes over a period of 8 minutes. The surface showed a finely fused, thin surface coating having a greenish tinge. After rinsing in plain water the coated panel was exposed to salt spray testing, as described above. After 167 hours in the salt spray chamber, the coated surface showed no corrosion. After 1,456 hours in the salt spray chamber the coated panel showed 15% corrosion.

#### EXAMPLE 9

Utilizing the same magnesium alloy and the same pretreatment with a solution of hydrofluoric acid, as described in Example 4, the magnesium panel was spark anodized utilizing an electrolyte containing 27.5 grams per liter of sodium fluoroborate, 25 grams per liter of potassium hydroxide, and 80 grams per liter of sodium hydroxide. Spark anodization was carried out at a potential of 55 to 60 volts and 5 to 7 amperes over a period of 8 minutes. Thereafter a potential of 62 volts and 10 to 13 amperes were applied over a period of 3 minutes. The appearance of the coating was white, uniform and tough. After rinsing the coating in plain water the coated magnesium panel was exposed to testing in the salt spray chamber, as described above, for a period of 167 hours. Evaluation thereafter showed no surface corrosion. After a total of 2,180 hours the sample showed less than 10% corrosion.

#### EXAMPLE 10

Utilizing the same magnesium alloy and the same pretreatment in an aqueous solution of hydrofluoric acid, as described in Example 4, a magnesium alloy panel was spark anodized utilizing an electrolyte solution containing 35.9 grams per liter of  $Na_3Fe(C_2O_4)$ , 40 grams per liter of potassium hydroxide and 5 grams per liter of sodium fluoroaluminate. The potential applied

to form a coating was 85 volts and 4 to 8 amperes over a period of 5 minutes. After rinsing the sample in plain water it was exposed to the salt spray chamber, as described above, for a period of 167 hours after which it was noted that less than 0.5% of the coated sample showed corrosion. After a total of 3,360 hours the coated sample showed about 20% corrosion.

While this invention has been described with reference to certain specific embodiments, it will be recognized by those skilled in the art that many variations are possible without departing from the scope and spirit of the invention, and it will be understood that it is intended to cover all changes and modifications of the invention disclosed herein for the purposes of illustration which do not constitute departures from the spirit and scope of the invention.

The embodiments of the invention in which an exclusive property or privilege is claimed are defined as follows:

1. An article consisting of a rectifier metal or alloy thereof coated with at least one anticorrosive coating by the process comprising:

(a) immersing said rectifier metal or alloy thereof in a strongly alkaline aqueous bath comprising at least one water soluble iron salt selected from the group consisting of at least one of the water soluble fluoroborates, fluorosilicates, and fluoroaluminates, and

(b) establishing a potential difference of at least 50 volts between said rectifier metal article or alloy thereof as an anode and a cathode in said bath to deposit said coating on said metal or alloy thereof.

2. An article according to claim 1 wherein the thickness of said anticorrosive coating is about 0.001 millimeter to about 2 millimeters.

3. An article according to claim 1 wherein the rectifier metal or alloy thereof is selected from the group consisting of aluminum and its alloys, beryllium and its alloys, magnesium and its alloys, tantalum and its alloys, tellurium and its alloys, silicon and its alloys, germanium and its alloys, titanium and its alloys, niobium and its alloys, calcium and its alloys and mixtures thereof.

4. An article according to claim 1 wherein the rectifier metal or alloy thereof is selected from the group consisting of magnesium and its alloys and aluminum and its alloys, said aqueous bath is maintained at a temperature of about 30° to about 90° centigrade, and said rectifier metal or alloy thereof is pretreated prior to coating by contacting an aqueous solution comprising hydrofluoric acid or an aqueous solution comprising a fluoride salt.

5. An article according to claim 4 wherein said rectifier metal alloy is a magnesium based alloy consisting of magnesium 90, aluminum 9, and zinc 1 and said water soluble salt is selected from the group consisting of ammonium and alkali metal fluoroborates, ammonium and alkali metal fluoroaluminates, ammonium and alkali metal fluorosilicates, and mixtures thereof.

6. The article of claim 4 wherein said rectifier metal alloy is a magnesium based alloy consisting of magnesium 90, aluminum 9, and zinc 1 and said water soluble iron salt is selected from the group consisting of ammonium or alkali metal ion cyanides, ammonium or alkali metal iron oxalates, and mixtures thereof.

7. A process of applying to a rectifier metal or alloy thereof at least one coating having improved resistance to corrosion by exposure to aqueous sodium chloride, said process comprising:

(a) contacting said rectifier metal or alloy thereof with a strongly alkaline aqueous bath comprising at least one water soluble iron salt or at least one salt selected from the group consisting of water soluble fluoroborates, fluorosilicates, and fluoroaluminates,

(b) applying an electrical potential of about 50 to about 1,000 volts between said metal utilized as an anode immersed in said aqueous bath and a cathode immersed in said aqueous bath, said electrical potential being maintained until the desired coating thickness is formed on said metal.

8. The process of claim 7 wherein said rectifier metal or alloy thereof is a metal or alloy thereof selected from at least one of the metals consisting of aluminum, beryllium, magnesium, tantalum, tellurium, silicon, germanium, titanium, niobium, or calcium and said bath is maintained at a temperature of about 30° to about 90° centigrade.

9. The process of claim 7 wherein said rectifier metal or alloy thereof is selected from the group consisting of magnesium, aluminum, and their alloys and said aqueous bath contains about 5 to about 150 grams per liter of said water soluble salt or mixtures thereof.

10. The process of claim 9 wherein said electrical potential is a direct current potential.

11. The process of claim 10 wherein said aqueous bath is made strongly alkaline utilizing an alkali metal

hydroxide, said bath is maintained at a temperature of about 50° to about 60° centigrade, and said metal or alloy thereof is pretreated prior to coating by contacting an aqueous solution comprising hydrofluoric acid or contacting an aqueous solution comprising a fluoride salt.

12. The process of claim 11 wherein said cathode is selected from the group consisting of iron and stainless steel.

13. The process of claim 12 wherein said rectifier metal alloy is a magnesium based alloy consisting of magnesium 90, aluminum 9, and zinc 1 and said water soluble salt is selected from the group consisting of ammonium and alkali metal fluoroborates, ammonium and alkali metal fluoroaluminates, ammonium and alkali metal fluorosilicates, and mixtures thereof.

14. The process of claim 12 wherein said rectifier metal alloy is a magnesium based alloy consisting of magnesium 90, aluminum 9, and zinc 1 and said water soluble iron salt is selected from the group consisting of an ammonium or an alkali metal iron cyanide, an ammonium or an alkali metal iron oxalate, and mixtures thereof.

15. The process of claim 14 wherein said alkali metal hydroxide is selected from the group consisting of sodium hydroxide, potassium hydroxide, and mixtures thereof.

\* \* \* \* \*

UNITED STATES PATENT AND TRADEMARK OFFICE  
CERTIFICATE OF CORRECTION

PATENT NO. : 4,668,347

DATED : May 26, 1987

INVENTOR(S) : Clarence E. Habermann and David S. Garrett

It is certified that error appears in the above-identified patent and that said Letters Patent is hereby corrected as shown below:

Col. 2, line 12; change "theof" to --thereof--.

Col. 6, line 1; change "estent" to --extent--.

Col. 6, line 49; change "path" to --bath--.

Col. 7, line 65; change "elecolyte" to --electrolyte--.

Col. 8, line 25, Claim 1; insert --or a salt-- before "selected".

Col. 8, line 63, Claim 6; change "ion" to --iron--.

Signed and Sealed this

Twenty-sixth Day of January, 1988

*Attest:*

DONALD J. QUIGG

*Attesting Officer*

*Commissioner of Patents and Trademarks*